

1

2,703,282

## INCREASING THE EXPOSURE LATITUDE OF PHOTOGRAPHIC EMULSIONS BY SENSITIZING

Burt H. Carroll, Rochester, N. Y., assignor to Eastman Kodak Company, Rochester, N. Y., a corporation of New Jersey

No Drawing. Application December 14, 1950,  
Serial No. 200,865

## 1 Claim. (Cl. 95—7)

This invention relates to photography and particularly to a method of sensitizing silver halide emulsions to increase latitude.

Latitude as used in photographic terminology is the distance along the exposure axis of the characteristic curve in which an increase in exposure produces a substantially uniform increase in density, that is, it is the projected distance along the exposure axis of the straight line portion of the characteristic curve (Mees, Theory of Photographic Process (1942) page 701). In the present case, latitude was measured as the distance along the exposure axis between the points where the gamma of the characteristic curve was 0.3 in the toe and 0.6 in the shoulder.

Total scale is defined as the distance along the exposure axis of the characteristic curve, between the extreme ends, that is, the toe and shoulder of the characteristic curve. This includes regions of under- and over-exposure (Mees, supra, page 703).

Speed of the photographic material is expressed for present purposes as the reciprocal of the inertia of the material, that is,

$$S = \frac{k}{i}$$

where  $k$  is a constant and  $i$  is the inertia.

Gamma is the tangent of the angle between the straight line portion of the characteristic curve and the exposure axis (Mees, supra, page 700).

It is well known that silver halide emulsions of different speeds may be blended to increase latitude (Nebblette, Brehm and Priest, "Elementary Photography" (1942), pages 190 and 191). Emulsions of different speeds may also be coated in separate layers for the same purpose. This arrangement always has the probability that development rates of the emulsions will not be the same so that the characteristic curve will be distorted except under a single development condition.

It is therefore an object of the present invention to provide a method for increasing the latitude of a photographic emulsion. A further object is to provide a method for increasing latitude without seriously changing the gamma or otherwise distorting the characteristic curve. Other objects will appear from the following description of my invention.

These objects are accomplished by sensitizing different portions of an emulsion with different optical sensitizers for the same spectral region and then mixing the portions so sensitized.

In general, my method of increasing latitude comprises sensitizing a silver halide emulsion, for example, a silver bromide or silver chlorobromide emulsion, with an optical sensitizing dye, sensitizing another portion of the same emulsion with a different optical sensitizing dye for the same spectral region but which gives a different speed, and mixing the two emulsions. By sensitizing "for the same region" I mean that the sensitizing maxima should not be more than about 25 millimicrons apart. The gammas of the two emulsions should usually be approximately the same but not necessarily so.

One of the emulsions may be present in any proportion from 25% to 80% of the mixture. More than two emulsions may be sensitized and mixed according to my invention but the mixture should comprise not less than

2

about 25% of any one emulsion. It is also possible to coat the emulsions as separate layers rather than mixing them and coating as a single layer.

My method of sensitizing differs from super-sensitizing in that the optical sensitizers may, and normally will, each sensitize as though the other were not present. The existence of super-sensitizing action of one or the other would not, however, prevent the use of my method; it will very rarely occur, however, since almost all of each of the dyes must remain on the grains to which they were originally added. My method differs from emulsions designed to give variable contrast (U. S. Patent 2,384,598) in that the two sensitizers used must sensitize for the same spectral region.

It is obvious that the optical sensitizing dye used according to my invention should be relatively non-diffusing since the dyes must be retained on the silver halide grains to which they are originally attached. Dyes of the following classes are suitable for use according to my invention.

- (1) Carbocyanines derived from  $\beta$ -naphthothiazole substituted in the central position of the chain by alkyl or aryl groups (Brooker U. S. Patent 1,846,301). These include  
3,3'-dimethyl-9-ethyl-4,5,4',5'-dibenzthiacarbo-cyanine chloride  
3,3'-dimethyl-9-phenyl-4,5,4',5'-dibenzthiacarbo-cyanine bromide  
3,3',9-triethyl-4,5,4',5'-dibenzthiacarbocyanine bromide

Corresponding dyes from  $\beta$ -naphthothiazole nuclei substituted in the nucleus by halogen, alkyl or alkoxy may also be used. The alkyl groups on the 3-positions may be replaced by hydroxyalkyl or carboxyalkyl, and the aryl group in the 9-position may be substituted by alkyl, halogen or alkoxy. These are red sensitizers.

(2) Carbocyanines derived from substituted benzothiazole or benzoselenazole substituted in the central position of the chain by alkyl or aryl groups, for example, 3,3',9-triethyl-5,5'-dichloroselenacarbocyanine bromide (made by the method of White U. S. 1,990,681 using 5-chloro-2-methyl-benzoselenazole instead of 2-methyl benzoselenazole). These are red sensitizers.

(3) 3,3'-dimethyl-8,10-aryloxythiocaboxyanines and oxacarbocyanines (Brooker and White U. S. Patent 2,478,366). These include 3,3'-dimethyl-8,10-m-tolox-thiocabocyanine bromide and 3,3'-dimethyl-8,10-m-toloxocabocyanine bromide. These are red and green sensitizers, respectively.

(4) Carbocyanines derived from 5-phenyl benzoxazole and 5-(p-tolyl) benzoxazole substituted in the central position of the chain by alkyl or aryl groups, for example, 3,3',9-triethyl-5,5'-diphenyl oxacarbocyanine bromide (See British Patent 496,116). These are green sensitizers.

(5) Complex merocyanines of U. S. Patent 2,454,629.

(6) Merocyanines derived from 1-benzothiazolyl-5-pyrazolone, such as those disclosed in Brooker U. S. Patent 2,211,762.

The optical sensitizing dyes are used according to my invention at a concentration of from about 4 to 50 milligrams of sensitizing dye per liter of emulsion containing about 0.25 gram mole of silver halide per liter of emulsion, the preferred concentration varying with the dye and with the grain size of the emulsion in accordance with normal sensitizing practice. An excess of dye is to be avoided because it leaves unabsorbed dye which diffuses to grains carrying the other dye.

The sensitizing dyes of groups 1 to 4 above, have the following structure:



where

Z and Z' = the atoms necessary to complete a  $\beta$ -naphthothiazole, 5-aryl benzoxazole or 5-aryl benzothiazole ring,

R and R<sub>1</sub> = alkyl,  
R<sub>3</sub> = hydrogen, alkyl or aryl,

$R_2$  and  $R_4$ =hydrogen and aryloxy,  
 $R_3$  being hydrogen when  $R_2$  and  $R_4$  are aryloxy, and  $R_2$  and  $R_4$  being hydrogen when  $R_3$  is alkyl or aryl.

The following table illustrates the increase in latitude which may be accomplished by blending suitable sensitized emulsions according to my invention.

|            | Speed | Gamma | Latitude |
|------------|-------|-------|----------|
| Emulsion 1 | 130   | 3.40  | 19       |
| Emulsion 2 | 15    | 3.70  | 10       |
| Blend      | 113   | 2.35  | 55       |
| Emulsion 1 | 63    | 3.46  | 12.5     |
| Emulsion 2 | 19    | 3.82  | 16       |
| Blend      | 5.4   | 2.45  | 40       |

My invention will now be described by reference to the following specific examples.

#### Example 1

A gelatino-silver chlorobromide emulsion containing  $\frac{1}{4}$  gram mole of silver chlorobromide per liter was divided into two equal portions. To one portion there was added an alcoholic solution of the red sensitizer 3,3'-dimethyl-9-ethyl-4,5,4',5'-dibenzthiacyarbocyanine chloride, 0.058 gram of sensitizer per mole of silver halide being used. The emulsion was digested for about five minutes at 50° C. with the dye. A portion of this emulsion was cooled to the coating temperature of approximately 38° C. coated and tested. Characteristics to red light exposure were found to be

10/i      Speed 130  
             Gamma 3.40  
             Latitude 19

To the second portion of emulsion there was added an alcoholic solution of the red sensitizer 3,3'-dimethyl-9-phenyl-4,5,4',5'-dibenzthiacyarbocyanine chloride, 0.058 gram of sensitizer being added per mole of silver halide. The emulsion was digested at 50° C. and a portion was cooled to 38° C., coated and tested. Characteristics to red light exposure were found to be

10/i      Speed 15  
             Gamma 3.70  
             Latitude 10

The remaining portions of both emulsions were cooled to the coating temperature of 38° C. and blended and coated without delay. The characteristics of the blend on exposure to red light were found to be

10/i      Speed 113  
             Gamma 2.35  
             Latitude 55 or more

#### Example 2

Two portions of the chlorobromide emulsion used in Example 1 were separately sensitized as described in Example 1 with different optical sensitizing dyes. One-half of the emulsion was sensitized with the green sensitizer 3,3',9 - triethyl - 5,5' - diphenyl - oxacarbocyanine bromide, 0.078 gram of sensitizer being used per mole of silver halide and the other half of the emulsion was sensitized with the green sensitizer 1 - (2 - benzothiazolyl) - 3 - methyl - 4 - [1 - methyl - 2(1) -  $\beta$  - naphthothiazolylidene] - 1 - ethylethylidene] - 5 - pyrazolone (see U. S. Patent 2,231,659, Example 15), 0.029 gram of sensitizer being used per mole of silver halide.

Upon coating and testing the emulsions separately, the portion sensitized with the first-mentioned dye when exposed through a Wratten Filter No. 12 transmitting light of about 500 to about 700 millimicron wave length was found to have a speed of 63, gamma of 3.46 and latitude of 12.5. The portion sensitized with the second-mentioned dye when exposed and processed in the same way was found to have a speed of 19, gamma of 3.82 and latitude of about 16. After blending the emulsions, the blend when exposed and processed in the same way was found to have a speed of 54, gamma of 2.45 and latitude of 40 or more.

#### Example 3

A portion of the emulsion sensitized to red light as described in Example 1 was mixed with an equal amount of the emulsion sensitized to green light as described in

Example 2, and the mixture was coated directly after mixing.

After drying, the coating was exposed to a color chart and was processed as follows, all of the solutions being at 68° F.:

(1) Prehardened in the following solution for 3 minutes:

|    |                             |       |     |
|----|-----------------------------|-------|-----|
| 10 | Sodium hexametaphosphate    | grams | 0.5 |
|    | Sodium bisulfite            | do    | 10  |
|    | Formaldehyde (40% solution) | cc    | 27  |
|    | Sodium carbonate            | grams | 10  |
|    | Sodium sulfate              | do    | 100 |
|    | Potassium bromide           | do    | 2.5 |
|    | Water to 1 liter.           |       |     |

(2) Washed for four minutes.

(3) Developed in a black and white developer of the following composition for 8 minutes:

|    |                                |       |      |
|----|--------------------------------|-------|------|
| 20 | Sodium hexametaphosphate       | grams | 0.5  |
|    | Sodium sulfide                 | do    | 40   |
|    | N-methyl-p-aminophenol sulfate | do    | 5.5  |
|    | Hydroquinone                   | do    | 2.2  |
| 25 | Sodium metaborate              | do    | 25   |
|    | Sodium thiocyanate             | do    | 0.45 |
|    | Potassium bromide              | do    | 4.5  |
|    | 6-nitrobenzimidazole           | do    | .02  |
|    | Water to 1 liter.              |       |      |

(4) Washed for 10 minutes.

(5) Reexposed to red light through a Wratten No. 70 filter.

(6) Developed in a cyan developer of the following composition for 15 minutes:

|    |                                                 |       |      |
|----|-------------------------------------------------|-------|------|
| 35 | Sodium hexametaphosphate                        | grams | 0.5  |
|    | Sodium sulfite                                  | do    | 5    |
|    | 2-amino-5-diethylaminotoluene hydrochloride     | do    | 2.8  |
|    | Sodium carbonate                                | do    | 15   |
| 40 | Potassium bromide                               | do    | 1.5  |
|    | 6-nitrobenzimidazole                            | do    | 0.15 |
|    | 2,4-dichloro-5-p-toluene sulfonamino-1-naphthol | do    | 0.4  |
|    | Sodium hydroxide                                | do    | 2.   |
|    | Water to 1 liter.                               |       |      |

(7) Washed for two minutes.

(8) Developed in an auxiliary black and white developer for three minutes. This developer had the same composition as developer 3, except that it contained no sodium thiocyanate.

(9) Washed for 10 minutes.

(10) Re-exposed to green light through a Wratten No. 16 filter.

(11) Developed for 15 minutes in a magenta developer of the following composition:

|    |                                         |       |     |
|----|-----------------------------------------|-------|-----|
| 55 | Sodium hexametaphosphate                | grams | 0.5 |
|    | Sodium sulfite                          | do    | 5   |
|    | 2-amino-5-diethyl toluene hydrochloride | do    | 2   |
|    | Sodium carbonate                        | do    | 20  |
| 60 | Potassium bromide                       | do    | 1   |
|    | 6-nitrobenzimidazole                    | do    | .01 |
|    | 2-cyanoacetyl coumarone                 | do    | 2.5 |
|    | Sodium hydroxide                        | do    | 2   |
|    | Water to 1 liter.                       |       |     |

(12) Washed for 10 minutes.

(13) Treated for four minutes in the following ferrocyanide bath:

|    |                          |       |    |
|----|--------------------------|-------|----|
| 70 | Sodium hexametaphosphate | grams | 1  |
|    | Potassium ferricyanide   | do    | 80 |
|    | Potassium bromide        | do    | 40 |
|    | Water to 1 liter.        |       |    |

(14) Fixed for two minutes in the following bath:

|    |                          |       |     |
|----|--------------------------|-------|-----|
| 75 | Sodium hexametaphosphate | grams | 10  |
|    | Sodium sulfite           | do    | 10  |
|    | Sodium thiosulfate       | do    | 320 |
|    | Water to 1 liter.        |       |     |

(15) Washed for 20 minutes.

The image thus produced was satisfactory from the standpoint of color separation and image quality.

It is apparent that my method has resulted in a substantial increase in the latitude of the blended emulsion.

This method is useful in producing either black and white or color emulsions. It is especially useful in mixed grain processes of color photography where two or more batches of silver halide sensitive to spectral regions are incorporated in the same emulsion layer. In such cases it is desirable to have sufficient latitude in each of the different spectral regions so that the exposure light in the various spectral regions can be balanced to produce images having similar characteristic curves. The advantage in freedom from differences in development rate of the blended emulsions is obvious. My method also provides a blending procedure which is uniformly reproducible from emulsion to emulsion.

Where I refer in the claims to sensitizing for a spectral region "of longer wave length than that which is appreciably absorbed by said emulsion," I mean sensitizing for longer wave length than about 500 millimicrons in the case of a silver bromoiodide emulsion, about 450 millimicrons in the case of a pure silver bromide emulsion, or about 400 millimicrons in the case of a pure silver chloride emulsion; that is, the sensitizing should be for a longer wave length than the natural sensitivity or absorption of the emulsion.

It will be understood that my invention is to be taken as limited only by the scope of the appended claim.

I claim:

The method of increasing the exposure latitude of a

gelatino-silver halide emulsion, which comprises dividing said emulsion into two approximately equal parts, sensitizing one part of said emulsion to red light with a 3,3'-dimethyl-9-ethyl-4,5,4',5'-dibenzthiacarbocyanine salt, sensitizing the other part of said emulsion to red light with a 3,3'-dimethyl-9-phenyl-4,5,4',5'-dibenzthiacarbocyanine salt, and mixing the parts so sensitized.

References Cited in the file of this patent

UNITED STATES PATENTS

|           |                  |                |
|-----------|------------------|----------------|
| 1,900,869 | Seymour          | Mar. 7, 1933   |
| 1,926,643 | Bialon           | Sept. 12, 1933 |
| 1,980,941 | Mannes et al.    | Nov. 13, 1934  |
| 2,029,946 | Schmid           | Feb. 4, 1936   |
| 2,295,276 | Willmanns et al. | Sept. 8, 1942  |
| 2,384,598 | Carroll          | Sept. 11, 1945 |
| 2,388,859 | Mannes et al.    | Nov. 13, 1945  |
| 2,620,272 | Schwarz          | Dec. 2, 1952   |

OTHER REFERENCES

Wall, Photographic Emulsions (1929), publ. by American Phot. Pub. Co., Boston; pp. 135-137.

Clerc, Photographic Theory and Practice, 2nd ed. (1937), publ. by Sir Isaac Pitman & Sons, Ltd., N. Y., p. 141.